# EUROPEAN PATENT SPECIFICATION

(11) **EP 3 981 526 B1**
(45) Date of publication and mention of the grant of the patent: **24.06.2026**
(21) Application number: 20836144.4
(22) Date of filing: 06.07.2020
(51) Int. Cl.: B22D 11/124, B22D 11/22

(54) **SECONDARY COOLING METHOD AND APPARATUS FOR CONTINUOUSLY CAST SLAB**
SEKUNDÄRKÜHLUNGSVERFAHREN UND -VORRICHTUNG FÜR STRANGGEGOSSENE PLATTEN
PROCÉDÉ ET APPAREIL DE REFROIDISSEMENT SECONDAIRE POUR DALLES COULÉES EN CONTINU

(30) Priority: 11.07.2019 JP 2019128853
(43) Date of publication of application: 13.04.2022
(73) Proprietor: JFE Steel Corporation, Tokyo 100-0011 (JP)
(72) Inventor: OSUKA Kenichi, Tokyo 100-0011 (JP); SUGIHARA Hirokazu, Tokyo 100-0011 (JP); UEOKA Satoshi, Tokyo 100-0011 (JP)
(74) Representative: Haseltine Lake Kempner LLP
(86) International application number: PCT/JP2020/026488
(87) International publication number: WO 2021/006254

(56) References cited:
- EP-A1- 3 932 586
- EP-A1- 3 998 126
- JP-A- 2008 212 972
- JP-A- 2008 254 062
- JP-A- 2014 200 803
- JP-A- 2018 015 781

## Description

### Technical Field

The present invention relates to a secondary cooling method and apparatus for a continuously cast slab.

### Background Art

A general method for manufacturing a continuously cast slab with vertical bending type continuous casting equipment, for example, will be described with reference to Figs. 3 and 4.

Molten steel poured into a mold 3 from a tundish (not illustrated) is subjected to first cooling by the mold 3 and formed into a flat plate-shaped cast slab 5 having a solidifying shell. The flat plate-shaped cast slab 5 moves downward through a vertical zone 9 and enters a curved zone 13. In a bending portion 11 provided at the entrance of the curved zone 13, the cast slab 5 is bent while being guided by a plurality of rollers (not illustrated) so that the curvature radius thereof is maintained constant.

After that, the cast slab 5 is unbent (straightened) in a straightening portion 15 such that the curvature radius thereof is gradually increased, and returns to the flat plate shape when the cast slab 5 moves out of the straightening portion 15 and into a horizontal zone 17. After being completely solidified in the horizontal zone 17, the cast slab 5 is cut to a predetermined length by a gas cutting machine 23 installed at the exit of a continuous casting machine.

The gas cutting machine 23 moves in a casting direction at a speed that matches a transport speed of the cast slab 5 while simultaneously moving a torch in a width direction. The gas cutting machine 23 discharges oxygen for cutting while heating the cast slab 5 with a preheating flame emitted from the torch, so that the cast slab 5 is melted and cut by oxidation heat of steel with oxygen.

When the casting speed is too high or when the cast slab temperature is too low, the cutting pitch of the gas cutting machine 23 cannot be synchronized with the casting speed. Therefore, a problem such as limitation to the casting speed or a cutting failure may occur. Accordingly, it is important to set a casting speed that matches the cutting performance and appropriately manage the temperature of the cast slab 5. The cast slab 5 cut by the gas cutting machine 23 is transported to a cast slab finishing plant or a rolling plant for the next process.

After leaving the mold 3, the cast slab 5 is subjected to secondary cooling for completely solidifying the cast slab 5 to a central portion thereof using water sprays (water-liquid sprays or water-air two-fluid mixture mist sprays) in a region from the vertical zone 9 to the horizontal zone 17.

In general, secondary cooling is performed by spraying water at a high flow rate in the vertical zone 9 that is directly below the mold 3, so that the cooling rate of the cast slab 5 is increased (in this specification, cooling of the cast slab at an increased cooling rate is referred to as "strong cooling") to ensure that the solidifying shell has a sufficient strength. In the curved zone 13 and the following zones, cooling of the cast slab 5 is reduced so that heat is conducted from a high-temperature region inside the cast slab 5 to increase the surface temperature of the cast slab 5 (heat recuperation). In the straightening portion 15, the surface temperature is adjusted to be above a brittle temperature range to avoid transversal cracking of the cast slab 5.

The cast slab 5 that has passed through the straightening portion 15 is completely solidified to the central portion thereof while being cooled in the horizontal zone 17. When the solidifying rate is low relative to the casting speed, there is a possibility that a solidification completion position will not be inside the continuous casting machine and that molten steel will flow out from the cut surface during gas cutting. This may cause severe damage, such as damage to the equipment or stoppage of the operation. When the solidification is completed too early, cooling water supplied after the completion of the solidification is wasted. In addition, the cast slab 5 is greatly reduced in temperature and cannot be easily cut, as described above. Thus, the productivity and production stability are greatly influenced by the settings of the cooling conditions in the horizontal zone 17.

Fig. 4 is a graph showing the result of numerical analysis for reproducing a temperature history of the cast slab 5 cast by a general continuous casting method according to the related art. The vertical axis represents the temperature, and the horizontal axis represents the distance from the meniscus (molten steel surface in the mold).

The reference signs of regions corresponding to the regions after the mold 3 illustrated in Fig. 3 are shown at the top of the graph.

In the graph, the solid line, the dashed line, and the one-dot chain line show the temperature histories at the center of the surface of the cast slab in the width direction, corner portions of the cast slab (corner portions), and the center of the cross section of the cast slab, respectively. In addition, in the graph, the thin dashed line shows the minimum temperature at which cutting can be performed. Cutting can be performed in a temperature region above this temperature (see the arrows). In addition, in the graph, the solidification completion position is denoted by A, and the end of the continuous casting machine is denoted by B.

As is clear from the temperature history at the center of the surface of the cast slab in the width direction, in the vertical zone 9 directly below the mold 3, strong cooling at a high flow rate is performed by using water sprays to increase the shell thickness. Subsequently, in the bending portion 11 and the curved zone 13, the cooling rate is reduced so that heat is recuperated from the inside of the cast slab and that the surface temperature of the cast slab is controlled to be above a brittle temperature range 25 when the cast slab passes through the straightening portion 15. As a result, the cast slab 5 with satisfactory surface quality can be obtained.

The cast slab is also continuously cooled in the horizontal zone 17. When the central portion of the cast slab is completely solidified at point A, the temperature drop at the central portion of the cast slab increases. Then, the cast slab passes through the end of the continuous casting machine at point B, is cut to a predetermined length by the gas cutting machine 23, and is transported for the next process. In this example, the solidification completion position is sufficiently upstream of the end of the continuous casting machine, and the corner temperature of the cast slab is sufficiently higher than the temperature at which cutting can be performed. Therefore, the cast slab can be cut without any problem.

One problem that occurs during the above-described process of manufacturing the cast slab is a surface defect, such as longitudinal cracks and transverse cracks. The transverse cracks are characterized in being formed near the corner portions at the top surface of the cast slab in equipment such as a curved or vertical bending continuous casting machine in which straightening of the cast slab is performed. When the cast slab passes through the straightening portion while the temperature of the surface layer thereof is in the range of embrittlement of steel from the y low temperature range to the γ/α transformation temperature range (region III embrittlement), transverse cracks are formed due to tensile stress on the surface of the cast slab during the straightening process. Non Patent Literature 1, for example, describes that the transverse cracks can be prevented by slowing the secondary cooling of the cast slab and shifting away from the embrittlement range toward the high-temperature side during the straightening process.

In addition, Patent Literature 1 discloses a technology for preventing surface cracks by reducing the amount of cooling water for secondary cooling or stopping the cooling water at the final straightening point in the straightening portion, that is, at a position near the entrance of the horizontal zone so that heat is recuperated in the surface layer of the cast slab.

However, according to the method of shifting away from the brittle temperature toward the high temperature side, the average temperature at the cross section of the slab is increased at the exit of the straightening portion. As a result, the completion of solidification of the central portion of the cast slab is delayed. Therefore, to complete the solidification at a location inside the continuous casting machine, the length of the continuous casting machine may need to be increased. Alternatively, there is a possibility that the casting speed will be limited and the productivity will be impaired.

Patent Literature 2 discloses a technology of performing cooling with an adjustment cooling device provided in the horizontal zone located downstream of the straightening portion so that the solidification completion position is located inside the caster.

However, Patent Literature 2 does not refer to specific cooling conditions. Therefore, the surface temperature may be significantly uneven in the width direction depending on the cooling conditions, and there is a risk that surface cracks (longitudinal cracks) will be formed in the slab surface due to thermal stress caused by the uneven temperature distribution. There is also a risk that the solidification completion position will not be uniform in the width direction and the internal quality will vary.

Patent Literature 3 discloses a technology for reducing uneven cooling in secondary cooling. According to this technology, the stability of the cooling process can be increased by controlling the boiling state of water in a striking area of a water spray such that film boiling is maintained in a front stage part of a cooling zone and nucleate boiling is maintained in a rear stage part of the cooling zone.

In general, when the cooling conditions are constant in the width direction, the cooling rate is higher at the corner portions of the cast slab than at the central portion of the cast slab in the width direction because heat is also dissipated from the sides. When cooling is started in a film boiling state, the film boiling state may be changed to a nucleate boiling state in response to a reduction in the temperature of the cooled surface. Therefore, when an attempt is made to maintain the film boiling state as in Patent Literature 3, the film boiling state is changed to the nucleate boiling state first at the corner portions of the cast slab at which the temperature is rapidly reduced, and the temperature is more rapidly reduced. Such a sudden change in temperature causes surface cracks in the cast slab due to thermal stress. In addition, the temperature drop at the corner portions of the cast slab may cause problems such as degradation of cutting properties or an increase in cutting time at the gas cutting machine provided at the exit of the continuous casting machine. These problems are not discussed in Patent Literature 3, and a method for controlling the temperature at the exit of the continuous casting machine is not clear.

Patent Literature 4 discloses a technology for cutting the cast slab after preliminarily heating the corner portions of the cast slab to ensure satisfactory cutting properties at the gas cutting machine. However, when strong cooling in a nucleate boiling state is performed as described above, the temperature of the cast slab is greatly reduced, and the required preheating time is longer than usual. In addition, when the casting speed is increased in accordance with the thickness of the cast slab or the type of steel, there may be a case where the gas cutting speed is not sufficient and the casting speed needs to be limited or where a very large amount of energy is needed for preliminary heating.

Patent Literature 5 discloses a method for continuously casting steel to reduce center segregation that occurs in a slab. This document was cited under Art. 54(3) EPC.

Patent Literature 6 discloses a method for producing a high Ni-containing steel cast slab by continuous casting.

Patent Literature 7 discloses a secondary cooling device for a continuous casting machine for cooling a cast piece manufactured by a continuous casting mold.

### Citation List

### Patent Literature

PTL 1: Japanese Patent No. 4690995
PTL 2: Japanese Unexamined Patent Application Publication No. 62-064462
PTL 3: Japanese Patent No. 6079387
PTL 4: Japanese Patent No. 2605329
PTL 5: European Patent Application No. 3 932 586 A1
PTL 6: Japanese Patent Application Publication No. 2008 212972
PTL 7: Japanese Patent Application Publication No. 2008 254062

### Non Patent Literature

NPL 1: Ogibayashi et al., The Iron and Steel Institute-Joint Society on Iron and Steel Basic Research "Dynamic Behavior in Continuous Casting", l985, p184

### Summary of Invention

### Technical Problem

As discussed above, secondary cooling conditions under which the surface quality is satisfactory, the productivity is not impaired, and no large additional energy cost is required are not clear.

In light of the above-described problems, an object of the present invention is to provide a secondary cooling method and apparatus for a continuously cast slab with which satisfactory surface quality of the cast slab can be ensured without impairing the productivity and without large additional energy cost.

### Solution to Problem

(1) A secondary cooling method for a continuously cast slab according to the present invention is a method in which the cast slab is cooled by spraying cooling water onto the cast slab in a secondary cooling zone of a continuous casting machine including a vertical zone, a bending portion, a curved zone, a straightening portion, and a horizontal zone arranged in that order from an upstream side in a casting direction, the cast slab being completely solidified in a section extending to an end of the horizontal zone. An upstream section of the horizontal zone in the casting direction is set to serve as a strong water cooling section in which the cast slab is cooled by spraying the cooling water under conditions such that the sprayed cooling water is in a nucleate boiling state at all positions in a width direction on a surface of the cast slab, and a section of the horizontal zone that is located downstream of the strong water cooling section in the casting direction and that extends to the end of the horizontal zone is set to serve as a non-water-cooled section in which spraying of the cooling water is stopped, so that a surface temperature of the cast slab is increased in the casting direction in a region from an end of the strong water cooling section to the end of the horizontal zone and that the surface temperature of the cast slab is within a predetermined range at the end of the horizontal zone.

In the secondary cooling method for a continuously cast slab, the horizontal zone is divided into n sections (n is an integer, 3 ≤ n) in the casting direction such that n-i^{th} to n^{th} sections (i is an integer, 0 ≤ i < n-1) each serve as the non-water-cooled section and that 1^{st} to n-i-1^{th} sections each serve as the strong water cooling section. A flow density of the cooling water per unit time in 1^{st} to j^{th} sections (j is an integer, 1 ≤ j < n-i-1) among the 1^{st} to n-i-1^{th} sections that each serve as the strong water cooling section is greater than a flow density of the cooling water per unit time in j+1^{th} to n-i-1^{th} sections.

In the secondary cooling method for a continuously cast slab, the flow density of the cooling water in the 1^{st} to j^{th} sections (j is an integer, 1 ≤ j < n-i-1) among the 1^{st} to n-i-1^{th} sections that each serve as the strong water cooling section is 500 L/(m²·min) or more and may be 2000 L/(m²·min) or less (min means minute as a unit of time), and the flow density of the cooling water in the j+1^{th} to n-i-1^{th} sections is 50 L/(m²·min) or more and less than 500 L/(m²·min).

In the secondary cooling method for a continuously cast slab, the surface temperature of the cast slab at the end of the horizontal zone is 350°C or more at a position at which the surface temperature is minimum in the width direction of the cast slab.

(2) A secondary cooling apparatus for a continuously cast slab according to the present invention is an apparatus in which the cast slab is cooled by spraying cooling water onto the cast slab in a secondary cooling zone of a continuous casting machine including a vertical zone, a curved zone, and a horizontal zone arranged in that order from an upstream side in a casting direction, the cast slab being completely solidified in a section extending to an end of the horizontal zone. The horizontal zone is divided into n sections (n is an integer, 3 ≤ n) in the casting direction. The secondary cooling apparatus includes a plurality of spray nozzles, water supply means, and a water supply control device, the plurality of spray nozzles being disposed in respective ones of the sections of the horizontal zone, the water supply means and the water supply control device being capable of controlling spraying and stopping of the cooling water from the plurality of spray nozzles and a flow density of the cooling water per unit time for each of the sections. The water supply control device causes the spray nozzles to spray the cooling water in 1^{st} to n-i-1^{th} sections (i is an integer, 0 ≤ i < n-1) from an upstream side in the casting direction so that the 1^{st} to n-i-1^{th} sections each serve as a strong water cooling section in which the sprayed cooling water is in a nucleate boiling state at all positions in a width direction on a surface of the cast slab, and stops spraying of the cooling water from the spray nozzles in n-i^{th} to n^{th} sections (i is an integer, 0 ≤ i < n-1) so that the n-i^{th} to n^{th} sections each serve as a non-water-cooled section.

In the secondary cooling apparatus for a continuously cast slab, the water supply control device controls the spraying of the cooling water from the spray nozzles such that a flow density of the cooling water per unit time in 1^{st} to j^{th} sections (j is an integer, 1 ≤ j < n-i-1) among the 1^{st} to n-i-1^{th} sections that each serve as the strong water cooling section is greater than a flow density of the cooling water per unit time in j+1^{th} to n-i-1^{th} sections.

In the secondary cooling apparatus for a continuously cast slab, the water supply control device controls the spraying of the cooling water from the spray nozzles such that the flow density of the cooling water in the 1^{st} to j^{th} sections (j is an integer, 1 ≤ j < n-i-1) among the 1^{st} to n-i-1^{th} sections that each serve as the strong water cooling section is 500 L/(m²·min) or more, and that the flow density of the cooling water in the j+1^{th} to n-i-1^{th} sections is 50 L/(m²·min) or more and less than 500 L/(m²·min). The water supply control device may control the spraying of the cooling water from the spray nozzles such that the flow density of the cooling water in the 1^{st} to j^{th} sections is 2000 L/(m²·min) or less (min means minute as a unit of time).

### Advantageous Effects of Invention

According to the present invention, the upstream section of the horizontal zone in the casting direction is set to serve as the strong water cooling section in which the cast slab is cooled by spraying the cooling water under conditions such that the sprayed cooling water is in a nucleate boiling state at all positions in the width direction on the surface of the cast slab, and the section of the horizontal zone that is located downstream of the strong water cooling section in the casting direction and that extends to the end of the horizontal zone is set to serve as the non-water-cooled section in which spraying of the cooling water is stopped, so that the surface temperature of the cast slab is increased in the casting direction in a region from an end of the strong water cooling section to the end of the horizontal zone and that the surface temperature of the cast slab is within a predetermined range at the end of the horizontal zone. Therefore, satisfactory surface quality of the cast slab can be ensured without impairing the productivity and without large additional energy cost.

### Brief Description of Drawings

[Fig. 1] Fig. 1 illustrates the general structure of continuous casting equipment according to an embodiment of the present invention.
[Fig. 2] Fig. 2 is a graph showing the temperature history of a cast slab in a continuous casting method according to the embodiment of the present invention.
[Fig. 3] Fig. 3 illustrates the general structure of general continuous casting equipment according to the related art.
[Fig. 4] Fig. 4 is a graph showing the temperature history of a cast slab in a general continuous casting method according to the related art.

### Description of Embodiments

A continuous casting machine to which a secondary cooling method for a continuously cast slab according to the present embodiment is applied will be described with reference to Fig. 1.

As illustrated in Fig. 1, a continuous casting machine 1 is an apparatus in which molten steel poured into a mold 3 from a tundish (not illustrated) is pulled out in the form of a cast slab 5 while being supported by rollers (not illustrated) and subjected to secondary cooling performed by cooling sprays (not illustrated) disposed between the rollers.

As illustrated in Fig. 1, the cast slab 5 is subjected to secondary cooling in a secondary cooling zone 7 that is divided into a vertical zone 9, a bending portion 11, a curved zone 13, a straightening portion 15, and a horizontal zone 17. The secondary cooling method according to the present invention is characterized mainly by a method for cooling the cast slab 5 in the horizontal zone 17.

In the secondary cooling zone 7 of the continuous casting machine 1, the horizontal zone 17 is divided into n sections (n is an integer, 3 ≤ n) and is provided with strong cooling equipment 21 including water supply means and a water supply control device 19 by which cooling water can be turned on and off and the amount thereof can be controlled for each section.

Although the number, n, of sections is determined in advance depending on the equipment, which of the n sections is to serve as a strong water cooling section or as a non-cooled section may be set as appropriate by the water supply control device 19.

Depending on the size of the equipment, the horizontal zone 17 may include nearly 100 rollers arranged at predetermined intervals in a casting direction. Spray nozzles that discharge cooling water are disposed between the rollers. Multiple spray nozzles are arranged in a width direction of the cast slab in each of the regions between the rollers.

In the strong cooling equipment 21 according to the present embodiment, the horizontal zone 17 is divided into n sections by dividing the spray nozzles into groups, each group including the spray nozzles disposed between a plurality of rollers (for example, ten rollers) arranged in the casting direction.

Therefore, in each section, the cooling water can be discharged from the group of spray nozzles at a high flow rate to quickly change the boiling state of the cooling water to a stable nucleate boiling state.

In each section, the nozzles and pipes that are used, for example, are changeable so that the cooling water may be discharged not only at a high flow rate but also at a low flow rate.

The spray nozzles used herein are not limited to water-liquid sprays and may instead be, for example, water-air two-fluid mixture mist spray nozzles as long as the flow density per unit time may be set as described below.

According to a secondary cooling method for a continuously cast slab of the present embodiment, the cast slab 5 that is cast by the above-described continuous casting machine 1 is cooled by spraying cooling water onto the cast slab 5 in the secondary cooling zone 7 including the vertical zone 9, the bending portion 11, the curved zone 13, the straightening portion 15, and the horizontal zone 17. The cast slab 5 is completely solidified within a section extending to an end of the horizontal zone. An upstream section of the horizontal zone 17 in the casting direction is set to serve as a strong water cooling section in which the cast slab 5 is cooled by spraying the cooling water under conditions such that the sprayed cooling water is in a nucleate boiling state on the surface of the cast slab. In addition, a section of the horizontal zone 17 that is located downstream of the strong water cooling section in the casting direction and that extends to the end of the horizontal zone is set to serve as a non-water-cooled section in which spraying of the cooling water is stopped.

The surface temperature of the cast slab is increased in the casting direction in a region from an end of the strong water cooling section to the end of the horizontal zone, and the surface temperature of the cast slab is within a predetermined range at the end of the horizontal zone.

Fig. 2 illustrates the result of numerical analysis for reproducing a temperature history of the surface of the cast slab manufactured by using the above-described continuous casting machine 1. In Fig. 2, the solid line, the dashed line, and the one-dot chain line show the temperature histories at the center of the surface of the cast slab in the width direction, corner portions of the cast slab (corner portions), and the center of the cross section of the cast slab, respectively. The thin dashed line shows the minimum temperature at which cutting can be performed. In addition, in Fig. 2, the solidification completion position is denoted by A', and the end of the continuous casting machine is denoted by B. Fig. 2 also shows the solidification completion position A according to the related art illustrated in Fig. 4.

The cast slab 5 is cooled in a manner similar to that in the technology of the related art until the cast slab 5 moving from the position directly below the mold 3 passes through the straightening portion 15, so that the surface temperature of the cast slab 5 in the straightening portion 15 is higher than the brittle temperature range 25.

When the cast slab enters the horizontal zone 17 and cooling by the strong cooling equipment 21 is started, the water sprays in the first one of the regions between the rollers in the horizontal zone 17 and water sprays downstream thereof in the casting direction in the horizontal zone 17 discharge water at a high flow rate so that a nucleate boiling state that is uniform in the width direction is achieved. As a result, the temperatures at the center of the cast slab in the width direction and at the corner portions of the cast slab are simultaneously reduced to a temperature close to the water temperature and stabilized.

After that, strong cooling is continued so that the nucleate boiling state is maintained. After the cast slab is completely solidified at point A', the internal temperature thereof starts to drop. It is not necessary to perform cooling after the interior is completely solidified or when the interior is not yet completely solidified but the temperature is sufficiently low and it is certain that the solidification will be completed before the cast slab reaches the end of the caster. Therefore, spraying is stopped in a region including i+1 sections that are the n-i^{th} to n^{th} sections (i is an integer, 0 ≤ i < n-1) so that heat is recuperated on the surface of the cast slab after point C. As a result, the temperature of the corner portions of the cast slab reaches or exceeds the temperature at which cutting can be performed at point B, and the cast slab can be cut without any problem.

In general, the temperature of the cast slab 5 is often controlled in response to a variation in the casting speed by changing the flow rate of the cooling water. However, when the temperature is reduced to a temperature close to a room temperature by performing strong cooling to ensure sufficient stability of the cooling process as in the present invention, the flow rate cannot be controlled because nucleate boiling is to be maintained. Accordingly, as described above, cooling needs to be stopped in some of the cooling sections to adjust the cooling time and control the temperature at which cooling is finished.

According to the present invention, strong cooling is performed in the horizontal zone 17. Therefore, when the casting speed is the same as that in the related art, the solidification completion position A' is located upstream of the position A according to the related art in the continuous casting machine 1. Accordingly, the casting speed can be increased from that in the related art. When the casting speed is increased, the time in which the cast slab passes through the cooling zone is reduced, and the cooling time is shortened. Accordingly, the number i+1 of non-water-cooled sections in which cooling is stopped may be reduced to increase the length of a portion of the cooling zone in which cooling is performed, so that the solidification is reliably completed in the continuous casting machine 1.

When casting is started or ended, the casting speed is reduced. In such a case, the number i+1 of non-water-cooled sections may be increased so that the temperature of the corner portions of the cast slab does not fall below the temperature at which cutting can be performed due to a drop in the overall temperature of the cast slab 5.

Regarding the spraying conditions of the cooling water (flow density per unit time) according to the present invention, conditions under which nucleate boiling is achieved over the entire area in the width direction in a short time irrespective of manufacturing conditions, such as a variation in the casting speed and the type of steel, or equipment conditions, such as arrangement intervals between the sprays, have been studied. As a result, it has been found that the flow density per unit time needs to be 500 L/(m²·min) (min means minute as a unit of time) or more. The flow density per unit time is a value calculated by dividing the flow rate of the cooling water (L/min) in the cooling section by the area (m²) of the cooling section.

When the flow density per unit time is less than or equal to the above-mentioned value, a stable nucleate boiling state cannot be achieved when the cast slab 5 at a high temperature is cooled, and the time at which nucleate boiling is achieved greatly differs between the positions at which the temperature drop is large (for example, the corner portions of the cast slab) and the positions at which the temperature drop is small (for example, the center of the cast slab in the width direction). As a result, the temperature significantly varies in the width direction.

Depending on the equipment arrangement or the type of steel, heat is greatly recuperated in regions toward which the cooling water is not directly discharged from the water sprays (for example, regions at and around the positions directly below the guide rollers), and there is a possibility that a stable nucleate boiling state cannot be achieved. This may cause a large temperature variation. Such a temperature variation may lead to deformation of the cast slab 5 and defects such as cracks.

When nucleate boiling is achieved, the cast slab is cooled mainly by boiling, and dependency of the cooling capacity on the flow density per unit time is reduced. Accordingly, when the flow density per unit time is increased beyond 2000 L/(m²·min), the cooling capacity cannot be greatly increased. Also, the total amount of cooling water that is used becomes excessive, and the capital investment on the water treatment equipment is increased. Therefore, the flow density per unit time in the strong water cooling section is suitably in the range of 500 L/(m²·min) or more and 2000 L/m²·min) or less.

When the cast slab 5 enters the above-described strong water cooling section and the surface temperature of the cast slab is reduced by nucleate boiling, the nucleate boiling state can be reliably maintained even when the flow rate is not as high as 500 L/(m²·min) or more.

Therefore, when there is a limit to the total amount of cooling water that can be used in the continuous casting machine 1, the 1^{st} to j^{th} sections (j is an integer, 1 ≤ j ≤ n-i-1) of the strong water cooling sections may be set to serve as a high-flow-rate region in which the flow density per unit time is greater than or equal to 500 L/(m²·min), and the remaining j+1^{th} to n-i-1^{th} sections may be set to serve as a low-flow-rate region in which the flow density per unit time is as low as 50 L/(m²·min) or more and less than 500 L/(m²·min) because it is only necessary to maintain nucleate boiling. The number j of the sections set to serve as the high-flow-rate region may be any number in accordance with the manufacturing conditions, such as the type of steel and the thickness of the cast slab.

A temperature range in which satisfactory cutting properties can be ensured in the gas cutting machine at the exit of the continuous casting machine has also been studied. As a result, it has been found that the corner temperature of the cast slab needs to be controlled to be 350°C or more at a position immediately in front of the cutting machine. Therefore, the surface temperature of the cast slab at the end of the horizontal zone 17 is preferably 350°C or more at the position at which the surface temperature is minimum in the width direction of the cast slab.

As described above, according to the present embodiment, the strong cooling equipment 21 divides the horizontal zone 17 of the secondary cooling zone 7 into a plurality of sections so that the strong water cooling section, in which cooling is performed while the nucleate boiling state is maintained, and the non-cooled section, which is located downstream of the strong water cooling section in the casting direction and in which spraying of the cooling water is stopped, are provided. The ranges of these sections are variable depending on the conditions such as the casting speed. Therefore, the temperature at the time when casting is ended can be controlled without causing a significantly uneven temperature distribution on the surface.

Accordingly, the cast slab 5 can be manufactured at a high speed while a high surface quality thereof is maintained, and can be cut without any problem even when the casting conditions are changed. Thus, stable production of a high quality cast slab 5 can be realized while the high productivity of the cast slab 5 is maintained.

The non-cooled section located downstream of the strong water cooling section in the casting direction is a section in which spraying of the cooling water is stopped to stop active cooling of the cast slab. Needless to say, the non-cooled section includes a section in which the cooling water is caused to fall onto the surface of the cast slab without an intention of cooling the cast slab as long as spraying of the cooling water for actively cooling the cast slab is stopped as described above. For example, the non-cooled section includes a section in which liquid remaining in the pipes falls onto the surface of the cast slab or in which a very small amount of water is supplied to prevent clogging of the spray nozzles.

In the non-cooled section, in addition to stopping the spraying of the cooling water, the temperature of the corner portions of the cast slab, at which the surface temperature of the cast slab is easily reduced, may be maintained or increased by using auxiliary means, such as a heat retaining cover or an edge heater.

When the predetermined flow density per unit time cannot be achieved for some reason, such as an abnormality in the equipment caused by leakage from the pipes, and when the nucleate boiling state cannot be quickly achieved after the cast slab enters the strong water cooling section, it is necessary to reliably achieve and maintain the nucleate boiling state by increasing the flow rate while monitoring the boiling state.

When the cooling water that is in contact with the surface of the cast slab is boiled, the cooling water is vaporized and turns into water vapor, which condenses into observable steam (water smoke) in air. In the nucleate boiling state, the cooling water that comes into contact with the cast slab surface violently forms bubbles and generates a large amount of water vapor and a large amount of water smoke. In contrast, in the film boiling state, the boiling cooling water forms less bubbles, and the amounts of water vapor and water smoke that are generated are reduced. Accordingly, a camera is installed in each section, and the amount of water smoke that is generated is monitored visually or by measurement with a transmissometer. A threshold of the amount of generated water smoke that delineates between nucleate boiling and film boiling is experimentally determined in advance, and whether the nucleate boiling state is achieved in a certain section can be determined by checking whether the amount of generated water smoke exceeds the threshold. When the nucleate boiling state is not achieved, the flow rate of the cooling water is increased. Thus, the nucleate boiling state can be reliably achieved and maintained.

### Examples

The cast slab 5 was manufactured by using the continuous casting machine 1 (Fig. 1) according to the above-described embodiment, and effects of the present invention were verified. This will be further described below.

In these examples, the horizontal zone 17 was divided into twelve sections (n=12), and whether or not to perform spraying and the spraying flow rate were controlled for each section. The length of the continuous casting machine 1 was 45 m, and a thermometer for measuring the temperature distribution on the surface of the cast slab and the gas cutting machine 23 were provided at the end of the caster.

The cast slab 5 was manufactured under different manufacturing conditions, for example, different flow densities per unit time (L/(m²·min)) in the horizontal zone, casting speeds, and slab thicknesses. The occurrence of an uneven temperature distribution during cooling, an estimated solidification completion position in the caster, the corner temperature of the cast slab in the cutting process, and the surface quality after the casting process were evaluated.

The manufacturing conditions and the results of the evaluation are shown in Table 1 given below. In Table 1, Examples 1 to 7 are within the scope of the present invention, and Comparative Examples 1 to 8 are outside the scope of the present invention.

The solidification completion position was estimated in advance by numerical analysis. In some of the comparative examples, no cast slab was actually manufactured because there was a risk that the solidification completion position will not be inside the continuous casting machine 1 according to the result of the preliminary estimation.

The results shown in Table 1 will now be discussed for each group of comparative examples and examples that relate to each other.

### <Comparative Examples 1 and 2 and Examples 1 and 2>

In Comparative Examples 1 and 2 and Examples 1 and 2, the cast slab 5 having a thickness of 235 mm was manufactured by using the technology of the related art and the present invention.

In Comparative Example 1, the cast slab was manufactured under cooling conditions according to the related art (flow density per unit time was 10 L/(m²·min), and no cooling stop region was provided). In this example, stable film boiling was constantly maintained on the surface. Therefore, no uneven temperature distribution occurred, and no problems were found in the inspection of the surface of the cast slab after manufacture. The corner temperature of the cast slab in the cutting process was 580°C, and cutting was performed without any problem.

However, the casting speed was limited to 1.0 mpm at a maximum so that the solidification completion position (estimated to be at a position of 36 m) was inside the caster.

Accordingly, in Comparative Example 2, a case in which the casting speed was increased to 2.5 mpm to increase the productivity was studied. No cast slab was actually manufactured because the estimated solidification completion position was calculated to be outside the caster under these conditions. Thus, according to the related art, although the cast slab 5 with satisfactory surface quality can be manufactured, the casting speed is limited.

In contrast, in Example 1, the technology of the present invention was applied so that the flow density per unit time was set to 500 L/(m²·min) to perform strong cooling in the 1^{st} to 9^{th} sections and that the cooling water was stopped to adjust the surface temperature by heat recuperation in the 10^{th} to 12^{th} sections. Casting was performed at a casting speed increased to 2.5 mpm. As a result, a nucleate boiling state was achieved uniformly in the width direction by strong cooling, and no uneven temperature distribution occurred. The estimated solidification completion position was at 38 m and was sufficiently inside the caster, and therefore the cast slab was actually manufactured. As a result, the corner temperature of the cast slab in the cutting process was 420°C, which was lower than that in Comparative Example 1 but within the range in which cutting can be performed. Accordingly, cutting was performed without any problem. The surface of the cast slab was inspected after manufacture, and no cracks were found. Thus, it was possible to efficiently manufacture the cast slab 5 with satisfactory surface quality without any problem.

In Example 2, the technology of the present invention was applied so that the flow density per unit time was set to 2000 L/(m²·min) to perform strong cooling in a region of the 1^{st} to 10^{th} sections and that the cooling water was stopped in a region of the 11^{th} and 12^{th} sections. In this case, it was possible to further increase the casting speed to 3.5 mpm and efficiently manufacture the high quality cast slab 5 without any trouble in the cutting process or any problem in the surface quality.

### <Comparative Examples 3 and 4>

In Comparative Examples 3 and 4, the cooling conditions in the strong water cooling sections were changed from those in Example 1. In Comparative Example 3, no cooling stop region was provided, and the flow density per unit time was set to 500 L/(m²·min) to perform strong cooling in all of the sections. In this case, no uneven temperature distribution occurred due to cooling, and the solidification completion position was inside the caster. However, since strong cooling was performed for a long time and heat recuperation was insufficient at the end of the caster, the corner temperature of the cast slab in the cutting process was reduced to 320°C. As a result, emergency reduction in the casting speed was necessary because it took a long time to cut the cast slab and there was a risk that cutting cannot be completed within the operation range of the gas cutting machine 23. In addition, the significant change in the casting speed caused degradation of the surface quality and internal quality of the cast slab 5 that was being manufactured.

In Comparative Example 4, the flow density per unit time was set to 400 L/(m²·min) in the 1^{st} to 10^{th} sections, and the cooling water was stopped in the 11^{th} and 12^{th} sections. As a result, in the strong water cooling sections, no stable nucleate boiling state not achieved on the cast slab at some positions in the width direction at the above-described flow rate. Nucleate boiling was achieved first at the corner portions of the cast slab, at which a large temperature drop occurs, and a significant temperature difference occurred in the width direction. Therefore, surface cracks and internal cracks were formed in the cast slab, and the quality of the cast slab 5 was degraded.

### <Examples 3 and 4 and Comparative Examples 5 and 6>

In Examples 3 and 4 and Comparative Examples 5 and 6, the conditions were changed from those in Example 1 such that only the 1^{st} section of the strong water cooling sections was set to serve as a high-flow-rate region, and the flow rate was reduced in the 2^{nd} and the following sections.

In Example 3, the flow density per unit time was set to 500 L/(m²·min) in the 1^{st} section serving as the high-flow-rate section, and to 50 L/(m²·min) in the 2^{nd} to 11^{th} sections. In the 12^{th} section, the cooling water was stopped. In this case, the nucleate boiling state was achieved by cooling in the 1^{st} section of the strong water cooling sections, and was maintained without causing heat recuperation in the following sections. As a result, uneven cooling did not occur in the width direction. The solidification completion position was at 43 m, and was inside the caster. The corner temperature of the cast slab in the cutting process was 430°C, and cutting was performed without any problem. The surface of the cast slab was inspected after manufacture, and no cracks were found. Thus, it was possible to manufacture the cast slab 5 with satisfactory surface quality.

In Example 4, the flow density per unit time was reduced stepwise in the strong water cooling sections. Specifically, the flow density per unit time was set to 2000 L/(m²·min) in the 1^{st} section, 1000 L/(m²·min) in the 2^{nd} section, 500 L/(m²·min) in the 3^{rd} section, 100 L/(m²·min) in the 4^{th} and 5^{th} sections, and 50 L/(m²·min) in the 6^{th} to 10^{th} sections. The cooling water was stopped in the 11^{th} and 12^{th} sections. In this case, the nucleate boiling state was achieved by cooling in the 1^{st} section of the strong water cooling sections, and was maintained without causing heat recuperation in the following sections. As a result, uneven cooling did not occur in the width direction. The solidification completion position was at 40 **m,** and was inside the caster. The corner temperature of the cast slab in the cutting process was 370°C, and cutting was performed without any problem. The surface of the cast slab was inspected after manufacture, and no cracks were found. Thus, it was possible to manufacture the cast slab 5 with satisfactory surface quality.

In Comparative Example **5,** the flow density per unit time was set to 40 L/(m²·min) in the latter ones of the strong water cooling sections serving as the low-flow-rate region. As a result, nucleate boiling was not maintained and the temperature was increased at the center of the cast slab in the width direction where large heat recuperation occurred, and a significantly uneven temperature distribution occurred in the width direction. Although the solidification completion position was inside the caster, the slab was deformed due to the uneven temperature distribution in the width direction, and cracks were formed in the surface.

In Comparative Example 6, the flow density per unit time was set to 400 L/(m²·min) in the first one of the strong water cooling sections serving as the high-flow-rate region. As a result, the nucleate boiling state was not quickly achieved when the cast slab 5 entered the strong water cooling section, and the nucleate boiling state and the film boiling state were both present in the width direction. Therefore, the surface temperature was significantly uneven, and surface cracks were formed. In addition, due to uneven cooling, the solidification completion position was also uneven, and the internal quality was degraded.

### <Example 5>

Example 5 is an example in which the casting speed needed to be greatly reduced at, for example, the start and end of the casting process in Example 1. In this case, the casting speed was reduced to 2.0 mpm, and strong cooling was performed for a longer time. Accordingly, the non-water-cooled sections were increased to the 8^{th} to 12^{th} sections. As a result, uneven cooling did not occur, and the solidification completion position was at 35 m. The corner temperature of the cast slab in the cutting process was 460°C, and was within the range in which cutting can be performed. The surface of the cast slab was inspected after manufacture, and no cracks were found. Thus, it was possible to manufacture the cast slab 5 with satisfactory surface quality without any problem even when the casting speed was greatly changed.

### <Comparative Examples 7 and 8 and Examples 6 and 7>

In Comparative Example 7 and Example 6 and in Comparative Example 8 and Example 7, the slab thickness was changed to 260 mm and 200 mm, respectively. In Comparative Examples 7 and 8, the slab thickness was changed to 260 mm and 200 mm, respectively, under the cooling conditions according to the related art similar to those in Comparative Example 1.

In Comparative Example 7, the slab thickness was 260 mm. Since the slab thickness was greater than that in Comparative Example 1 and the temperature drop was reduced accordingly, the casting speed was reduced to 0.8 mpm so that the solidification completion position was inside the caster. In Comparative Example 8, the slab thickness was 200 mm. To prevent an unnecessary temperature drop after the completion of solidification of the central portion due to the reduction in the slab thickness compared to that in Comparative Example 1, the casting speed was increased to 2.0 mpm.

In Example 6, the slab thickness was 260 mm. Since the slab thickness was greater than that in Example 1 and the temperature drop was reduced accordingly, the strong water cooling sections were increased to the 1^{st} to 11^{th} sections without changing the casting speed. The flow density per unit time in the strong water cooling sections was the same as that in Example 1. As a result, uneven cooling did not occur, and the solidification completion position was at 42 m. The corner temperature of the cast slab in the cutting process was 440°C, and was within the range in which cutting can be performed. The surface of the cast slab was inspected after manufacture, and no cracks were found. Thus, even when the casting thickness was increased, it was possible to manufacture the cast slab 5 with satisfactory surface quality without any problem while the high casting speed was maintained.

In Example 7, the slab thickness was 200 mm. Since the slab thickness was less than that in Example 1 and the temperature drop was increased accordingly, the casting speed was increased to 3.0 mpm. The flow density per unit time in the strong water cooling sections was the same as that in Example 1, and the non-water-cooled sections were increased to the 9^{th} to 12^{th} sections. As a result, uneven cooling did not occur, and the solidification completion position was at 37 m. The corner temperature of the cast slab in the cutting process was 430°C, and was within the range in which cutting can be performed. The surface of the cast slab was inspected after manufacture, and no cracks were found. Thus, even when the casting thickness was reduced, it was possible to manufacture the cast slab 5 with satisfactory surface quality without any problem and without greatly reducing the casting speed.

Thus, according to the technology of the present invention, it is not necessary to greatly change the casting speed as in the related art even when the thickness of the cast slab is changed, and stable and efficient production of a high quality cast slab 5 can be realized.

As described above, an upstream section of the horizontal zone 17 in the casting direction is set to serve as a strong water cooling section in which the cast slab 5 is cooled by spraying the cooling water under conditions such that the sprayed cooling water is in a nucleate boiling state at all positions in the width direction on the surface of the cast slab. In addition, a section of the horizontal zone 17 that is located downstream of the strong water cooling section in the casting direction and that extends to the end of the horizontal zone is set to serve as a non-water-cooled section in which spraying of the cooling water is stopped. It has been verified that according to the above configuration, even when the casting conditions are changed, the cast slab 5 can be manufactured while the temperature thereof is maintained at a temperature that allows easy cutting without limitation to the casting speed or large additional energy cost for heating the cast slab 5.

### Reference Signs List

- 1: continuous casting machine
- 3: mold
- 5: cast slab
- 7: secondary cooling zone
- 9: vertical zone
- 11: bending portion
- 13: curved zone
- 15: straightening portion
- 17: horizontal zone
- 19: water supply control device
- 21: strong cooling equipment
- 23: gas cutting machine
- 25: brittle temperature range

## Claims

1. A secondary cooling method for a continuously cast slab (5) in which the cast slab is cooled by spraying cooling water onto the cast slab in a secondary cooling zone (7) of a continuous casting machine (1) including a vertical zone (9), a bending portion (11), a curved zone (13), a straightening portion (15), and a horizontal zone (17) arranged in that order from an upstream side in a casting direction, the cast slab (5) being completely solidified in a section extending to an end of the horizontal zone (17),
wherein an upstream section of the horizontal zone (17) in the casting direction is set to serve as a strong water cooling section in which the cast slab (5) is cooled by spraying the cooling water under conditions such that the sprayed cooling water is in a nucleate boiling state at all positions in a width direction on a surface of the cast slab (5), and a section of the horizontal zone (17) that is located downstream of the strong water cooling section in the casting direction and that extends to the end of the horizontal zone (17) is set to serve as a non-water-cooled section in which spraying of the cooling water is stopped, so that a surface temperature of the cast slab (5) is increased in the casting direction in a region from an end of the strong water cooling section to the end of the horizontal zone (17) and that the surface temperature of the cast slab (5) is within a predetermined range at the end of the horizontal zone (17), wherein the surface temperature of the cast slab (5) at the end of the horizontal zone (17) is 350°C or more at a position at which the surface temperature is minimum in the width direction of the cast slab (5),
wherein the horizontal zone (17) is divided into n sections, where n is an integer, 3 ≤ n, in the casting direction such that n-i^{th} to n^{th} sections, where i is an integer, 0 ≤ i < n-1, each serve as the non-water-cooled section and that 1^{st} to n-i-1^{th} sections each serve as the strong water cooling section, and
wherein a flow density of the cooling water per unit time in 1^{st} to j^{th} sections, where j is an integer, 1 ≤ j < n-i-1, among the 1^{st} to n-i-1^{th} sections that each serve as the strong water cooling section is greater than a flow density of the cooling water per unit time in j+1^{th} to n-i-1^{th} sections, and
wherein the flow density of the cooling water in the 1^{st} to j^{th} sections, where j is an integer, 1 ≤ j < **n-i-1,** among the 1^{st} to n-i-1^{th} sections that each serve as the strong water cooling section is 500 L/(m²·min) or more, where min means minute as a unit of time, and the flow density of the cooling water in the j+1^{th} to n-i-1^{th} sections is 50 L/(m²·min) or more and less than 500 L/(m²·min).

2. The secondary cooling method for a continuously cast slab (5) according to Claim 1, wherein the flow density of the cooling water in the 1^{st} to j^{th} sections is 2000 L/(m²·min) or less.

3. A secondary cooling apparatus for a continuously cast slab (5) in which the cast slab is cooled by spraying cooling water onto the cast slab in a secondary cooling zone (7) of a continuous casting machine (1) including a vertical zone (9), a curved zone (13), and a horizontal zone (17) arranged in that order from an upstream side in a casting direction, the cast slab (5) being completely solidified in a section extending to an end of the horizontal zone (17),
wherein the horizontal zone (17) is divided into n sections, where n is an integer, 3 ≤ n, in the casting direction,
wherein the secondary cooling apparatus comprises a plurality of spray nozzles, water supply means, and a water supply control device (19), the plurality of spray nozzles being disposed in respective ones of the sections of the horizontal zone (17), the water supply means and the water supply control device (19) being capable of controlling spraying and stopping of the cooling water from the plurality of spray nozzles and a flow density of the cooling water per unit time for each of the sections, and
wherein the water supply control device (19) causes the spray nozzles to spray the cooling water in 1^{st} to n-i-1^{th} sections, where i is an integer, 0 ≤ i < n-1, from an upstream side in the casting direction so that the 1^{st} to n-i-1^{th} sections each serve as a strong water cooling section in which the sprayed cooling water is in a nucleate boiling state at all positions in a width direction on a surface of the cast slab (5), and stops spraying of the cooling water from the spray nozzles in n-i^{th} to n^{th} sections, where i is an integer, 0 ≤ i < n-1, so that the n-i^{th} to n^{th} sections each serve as a non-water-cooled section,
wherein the water supply control device (19) controls the spraying of the cooling water from the spray nozzles such that a flow density of the cooling water per unit time in 1^{st} to j^{th} sections, where j is an integer, 1 ≤ j < n-i-1, among the 1^{st} to n-i-1^{th} sections that each serve as the strong water cooling section is greater than a flow density of the cooling water per unit time in j+1^{th} to n-i-1^{th} sections, and wherein the water supply control device (19) controls the spraying of the cooling water from the spray nozzles such that the flow density of the cooling water in the 1^{st} to j^{th} sections, where j is an integer, 1 ≤ j < n-i-1, among the 1^{st} to n-i-1^{th} sections that each serve as the strong water cooling section is 500 L/(m²·min) or more, where min means minute as a unit of time, and that the flow density of the cooling water in the j+1^{th} to n-i-1^{th} sections is 50 L/(m²·min) or more and less than 500 L/(m²·min).

4. The secondary cooling apparatus for a continuously cast slab (5) according to Claim 3, wherein the water supply control device (19) controls the spraying of the cooling water from the spray nozzles such that the flow density of the cooling water in the 1^{st} to j^{th} sections is 2000 L/(m²·min) or less.

## Patentansprüche

1. Sekundärkühlverfahren für eine stranggegossene Bramme (5), bei dem die Gussbramme durch Sprühen von Kühlwasser auf die Gussbramme in einer Sekundärkühlzone (7) einer Stranggießmaschine (1), die eine Vertikalzone (9), einen Biegebereich (11), eine Bogenzone (13), einen Richtbereich (15) und eine Horizontalzone (17), die in dieser Reihenfolge von einer stromaufwärtigen Seite in einer Gießrichtung angeordnet sind, beinhaltet, gekühlt wird, wobei die Gussbramme (5) in einem Abschnitt, der sich bis zu einem Ende der Horizontalzone (17) erstreckt, vollständig erstarrt ist,
wobei ein stromaufwärtiger Abschnitt der Horizontalzone (17) in der Gießrichtung dazu eingestellt ist, als ein Starkwasserkühlabschnitt zu dienen, in dem die Gussbramme (5) durch Sprühen des Kühlwassers unter Bedingungen gekühlt wird, bei denen sich das gesprühte Kühlwasser in einem Blasensiedezustand an allen Positionen in einer Breitenrichtung auf einer Oberfläche der Gussbramme (5) befindet, und ein Abschnitt der Horizontalzone (17), der sich stromabwärts des Starkwasserkühlabschnitts in der Gießrichtung befindet und der sich bis zum Ende der Horizontalzone (17) erstreckt, dazu eingestellt ist, als ein nicht wassergekühlter Abschnitt zu dienen, in dem Sprühen des Kühlwassers gestoppt ist, so dass eine Oberflächentemperatur der Gussbramme (5) in der Gießrichtung in einem Bereich von einem Ende des Starkwasserkühlabschnitts bis zum Ende der Horizontalzone (17) erhöht wird und dass die Oberflächentemperatur der Gussbramme (5) am Ende der Horizontalzone (17) innerhalb eines vorbestimmten Bereichs liegt, wobei die Oberflächentemperatur der Gussbramme (5) am Ende der Horizontalzone (17) 350 °C oder mehr an einer Position beträgt, an der die Oberflächentemperatur in der Breitenrichtung der Gussbramme (5) minimal ist,
wobei die Horizontalzone (17) in der Gießrichtung in n Abschnitte unterteilt ist, wobei n eine ganze Zahl ist, 3 ≤ n, derart, dass n-i^{te} bis n^{te} Abschnitte, wobei i eine ganze Zahl ist, 0 ≤ i < n-1, jeweils als der nicht wassergekühlte Abschnitt dienen und dass 1. bis n-i-1^{te} Abschnitte jeweils als der Starkwasserkühlabschnitt dienen, und
wobei eine Durchflussdichte des Kühlwassers pro Zeiteinheit in 1. bis j^{tem} Abschnitt, wobei j eine ganze Zahl ist, 1 ≤ j < n-i-1, unter den 1. bis n-i-1^{ten} Abschnitten, die jeweils als der Starkwasserkühlabschnitt dienen, größer ist als eine Durchflussdichte des Kühlwassers pro Zeiteinheit in j+1^{tem} bis n-i-1^{tem} Abschnitt, und
wobei die Durchflussdichte des Kühlwassers in den 1. bis j^{ten} Abschnitten, wobei j eine ganze Zahl ist, 1 ≤ j < n-i-1, unter den 1. bis n-i-1^{ten} Abschnitten, die jeweils als der Starkwasserkühlabschnitt dienen, 500 L/(m² ·min) oder mehr beträgt, wobei min Minute als Zeiteinheit bedeutet, und die Durchflussdichte des Kühlwassers in den j+1^{ten} bis n-i-1^{ten} Abschnitten 50 L/(m² ·min) oder mehr und weniger als 500 L/(m² ·min) beträgt.

2. Sekundärkühlverfahren für eine stranggegossene Bramme (5) nach Anspruch 1, wobei die Durchflussdichte des Kühlwassers in den 1. bis j^{ten} Abschnitten 2000 L/(m² ·min) oder weniger beträgt.

3. Sekundärkühleinrichtung für eine stranggegossene Bramme (5), bei der die Gussbramme durch Sprühen von Kühlwasser auf die Gussbramme in einer Sekundärkühlzone (7) einer Stranggießmaschine (1), die eine Vertikalzone (9), eine Bogenzone (13) und eine Horizontalzone (17), die in dieser Reihenfolge von einer stromaufwärtigen Seite in einer Gießrichtung angeordnet sind, beinhaltet, gekühlt wird, wobei die Gussbramme (5) in einem Abschnitt, der sich bis zu einem Ende der Horizontalzone (17) erstreckt, vollständig erstarrt ist,
wobei die Horizontalzone (17) in der Gießrichtung in n Abschnitte unterteilt ist, wobei n eine ganze Zahl ist, 3 ≤ n, wobei die Sekundärkühleinrichtung eine Vielzahl von Sprühdüsen, Wasserzufuhrmittel und eine Wasserzufuhrsteuervorrichtung (19) umfasst, wobei die Vielzahl von Sprühdüsen in jeweiligen der Abschnitte der Horizontalzone (17) angeordnet ist, wobei die Wasserzufuhrmittel und die Wasserzufuhrsteuervorrichtung (19) in der Lage sind, Sprühen und Stoppen des Kühlwassers aus der Vielzahl von Sprühdüsen und eine Durchflussdichte des Kühlwassers pro Zeiteinheit für jeden der Abschnitte zu steuern, und
wobei die Wasserzufuhrsteuervorrichtung (19) die Sprühdüsen veranlasst, das Kühlwasser in 1. bis n-i-1^{ten} Abschnitten, wobei i eine ganze Zahl ist, 0 ≤ i < n-1, von einer stromaufwärtigen Seite in der Gießrichtung zu sprühen, so dass die 1. bis n-i-1^{ten} Abschnitte jeweils als ein Starkwasserkühlabschnitt dienen, in dem sich das gesprühte Kühlwasser in einem Blasensiedezustand an allen Positionen in einer Breitenrichtung auf einer Oberfläche der Gussbramme (5) befindet, und Sprühen des Kühlwassers aus den Sprühdüsen in n-i^{tem} bis n^{tem} Abschnitt, wobei i eine ganze Zahl ist, 0 ≤ i < n-1, stoppt, so dass die n-i^{ten} bis n^{ten} Abschnitte jeweils als ein nicht wassergekühlter Abschnitt dienen,
wobei die Wasserzufuhrsteuervorrichtung (19) das Sprühen des Kühlwassers aus den Sprühdüsen derart steuert, dass eine Durchflussdichte des Kühlwassers pro Zeiteinheit in 1. bis j^{tem} Abschnitt, wobei j eine ganze Zahl ist, 1 ≤ j < n-i-1, unter den 1. bis n-i-1^{ten} Abschnitten, die jeweils als der Starkwasserkühlabschnitt dienen, größer ist als eine Durchflussdichte des Kühlwassers pro Zeiteinheit in j+1^{tem} bis n-i-1^{tem} Abschnitt, und wobei die Wasserzufuhrsteuervorrichtung (19) das Sprühen des Kühlwassers aus den Sprühdüsen derart steuert, dass die Durchflussdichte des Kühlwassers in den 1. bis j^{ten} Abschnitten, wobei j eine ganze Zahl ist, 1 ≤ j < n-i-1, unter den 1. bis n-i-1^{ten} Abschnitten, die jeweils als der Starkwasserkühlabschnitt dienen, 500 L/(m² ·min) oder mehr beträgt, wobei min Minute als Zeiteinheit bedeutet, und dass die Durchflussdichte des Kühlwassers in den j+1^{ten} bis n-i-1^{ten} Abschnitten 50 L/(m² ·min) oder mehr und weniger als 500 L/(m² ·min) beträgt.

4. Sekundärkühleinrichtung für eine stranggegossene Bramme (5) nach Anspruch 3, wobei die Wasserzufuhrsteuervorrichtung (19) das Sprühen des Kühlwassers aus den Sprühdüsen derart steuert, dass die Durchflussdichte des Kühlwassers in den 1. bis j^{ten} Abschnitten 2000 L/(m² ·min) oder weniger beträgt.

## Revendications

1. Procédé de refroidissement secondaire pour une brame coulée en continu (5) dans lequel la brame coulée est refroidie par pulvérisation d'eau de refroidissement sur la brame coulée dans une zone de refroidissement secondaire (7) d'une machine de coulée continue (1) comprenant une zone verticale (9), une zone de cintrage (11), une zone courbe (13), une zone de redressement (15) et une zone horizontale (17) disposées dans cet ordre à partir d'un côté en amont dans le sens de la coulée, la brame coulée (5) étant complètement solidifiée dans une section s'étendant jusqu'à une extrémité de la zone horizontale (17),
dans lequel une section amont de la zone horizontale (17), dans le sens de la coulée, est conçue pour servir de section de refroidissement par eau intense, dans laquelle la brame coulée (5) est refroidie par la pulvérisation de l'eau de refroidissement dans des conditions telles que l'eau de refroidissement pulvérisée soit dans un état d'ébullition nucléée à toutes les positions dans une direction de largeur sur une surface de la brame coulée (5), et une section de la zone horizontale (17) située en aval de la section de refroidissement par eau intense dans le sens de la coulée et s'étendant jusqu'à l'extrémité de la zone horizontale (17) est conçue pour servir de section non refroidie par eau, dans laquelle la pulvérisation de l'eau de refroidissement est arrêtée, de sorte qu'une température de surface de la brame coulée (5) soit augmentée dans le sens de la coulée dans une région allant de l'extrémité de la section de refroidissement par eau intense jusqu'à l'extrémité de la zone horizontale (17), et que la température de surface de la brame coulée (5) soit située dans une plage prédéterminée à l'extrémité de la zone horizontale (17), la température de surface de la brame coulée (5) à l'extrémité de la zone horizontale (17) étant de 350°C ou plus à une position à laquelle la température de surface est minimale dans le sens de la largeur de la brame coulée (5),
dans lequel la zone horizontale (17) est divisée en n sections, où n est un entier, 3 ≤ n, dans la direction de coulée, de sorte que les n-i^{e} à n^{e} sections, où i est un entier, 0 ≤ i < n-1, servent chacune de section non refroidie par eau et que les 1^{e} à n-i-1^{e} sections servent chacune de section de refroidissement par eau intense, et
dans lequel la densité de flux de l'eau de refroidissement par unité de temps dans les 1^{e} à j^{e} sections, où j est un entier, 1 ≤ j < ni-1, parmi les 1^{e} à n-i-1^{e} sections qui servent chacune de section de refroidissement par eau intense, est supérieure à la densité de flux de l'eau de refroidissement par unité de temps dans les j+1^{e} à n-i-1^{e} sections, et
dans lequel la densité de flux de l'eau de refroidissement dans les 1^{e} à j^{e} sections, où j est un entier, 1 ≤ j < ni-1, parmi les 1^{e} à n-i-1^{e} sections qui servent chacune de section de refroidissement par eau intense, est de 500 L/ (m² ·min) ou plus, où min signifie minute comme unité de temps, et la densité de flux de l'eau de refroidissement dans les j+1^{e} à n-i-1^{e} sections est de 50 L/ (m² ·min) ou plus et inférieure à 500 L/ (m² ·min).

2. Procédé de refroidissement secondaire pour une brame coulée en continu (5) selon la revendication 1, dans lequel la densité de flux de l'eau de refroidissement dans les 1^{e} à j^{e} sections est de 2000 L/ (m² ·min) ou moins.

3. Appareil de refroidissement secondaire pour une brame coulée en continu (5) dans lequel la brame coulée est refroidie par pulvérisation d'eau de refroidissement sur la brame coulée dans une zone de refroidissement secondaire (7) d'une machine de coulée continue (1) comprenant une zone verticale (9), une zone courbe (13) et une zone horizontale (17) disposées dans cet ordre à partir d'un côté en amont dans le sens de la coulée, la brame coulée (5) étant complètement solidifiée dans une section s'étendant jusqu'à une extrémité de la zone horizontale (17), dans lequel la zone horizontale (17) est divisée en n sections, où n est un entier, 3 ≤ n, dans la direction de coulée,
dans lequel l'appareil de refroidissement secondaire comprend une pluralité de buses de pulvérisation, des moyens d'alimentation en eau et un dispositif de contrôle de l'alimentation en eau (19), la pluralité de buses de pulvérisation étant disposées dans des sections respectives de la zone horizontale (17), les moyens d'alimentation en eau et le dispositif de contrôle de l'alimentation en eau (19) étant capables de contrôler la pulvérisation et l'arrêt de l'eau de refroidissement provenant des buses de pulvérisation ainsi que la densité de flux de l'eau de refroidissement par unité de temps pour chacune des sections, et
dans lequel le dispositif de contrôle d'alimentation en eau (19) provoque la pulvérisation d'eau de refroidissement à partir des buses de pulvérisation dans les 1^{e} à n-i-1^{e} sections, où i est un entier, 0 ≤ i < n-1, depuis un côté amont dans la direction de coulée de sorte que les 1^{e} à n-i-¹ sections servent chacune de section de refroidissement par eau intense dans laquelle l'eau de refroidissement pulvérisée est à l'état d'ébullition nucléée à toutes les positions dans le sens de la largeur sur une surface de la drame coulée (5), et arrête la pulvérisation d'eau de refroidissement à partir des buses de pulvérisation dans les n-i^{e}à n^{e} sections, où i est un entier, 0 ≤ i < n-1, de sorte que les n-i^{e} à n^{e} sections servent chacune de section non refroidie par l'eau,
dans lequel le dispositif de contrôle d'alimentation en eau (19) contrôle la pulvérisation de l'eau de refroidissement à partir des buses de pulvérisation de sorte que la densité de flux de l'eau de refroidissement par unité de temps dans les sections¹ à^{j}, où j est un entier, 1 ≤ j < ni-1, parmi les sections¹ à ni-¹ qui constituent chacune une section de refroidissement à eau forte, soit supérieur au débit massique d'eau de refroidissement par unité de temps dans les j+¹ à n-i-1^{e} sections, et dans lequel le dispositif de contrôle d'alimentation en eau (19) contrôle la pulvérisation de l'eau de refroidissement à partir des buses de pulvérisation de sorte que la densité de flux de l'eau de refroidissement dans les 1^{e} à j^{e} sections, où j est un entier, 1 ≤ j < ni-1, parmi les 1^{e} à n-i-1^{e} sections qui servent chacune de section de refroidissement par eau intense, soit de 500 L/(m² ·min) ou plus, où min signifie minute comme unité de temps, et que la densité de flux de l'eau de refroidissement dans les j+1^{e} à n-i-1^{e} sections soit de 50 L/ (m² ·min) ou plus et inférieure à 500 L/ (m² ·min).

4. Appareil de refroidissement secondaire pour une brame coulée en continu (5) selon la revendication 3, dans lequel le dispositif de contrôle d'alimentation en eau (19) contrôle la pulvérisation de l'eau de refroidissement à partir des buses de pulvérisation de sorte que la densité de flux de l'eau de refroidissement dans les 1^{e} à j^{e} sections soit de 2000 L/ (m² ·min) ou moins.
